

Cross Reference

Exam.

(No Model.)

J. MURPHY.

COBBLE STONE AND GROUT PAVEMENT.

No. 258,460.

Patented May 23, 1882.



WITNESSES:

*w. w. hillingsworth*  
*A. G. Lyne.*

INVENTOR:

*John Murphy*  
BY *John Murphy*

ATTORNEYS.

106  
—  
98

258,460

XR

UNITED STATES PATENT OFFICE.

JOHN MURPHY, OF COLUMBUS, OHIO.

COBBLE-STONE AND GROUT PAVEMENT.

SPECIFICATION forming part of Letters Patent No. 258,460, dated May 23, 1882.

Application filed February 11, 1882. (No model.)

*To all whom it may concern:*

Be it known that I, JOHN MURPHY, of Columbus, in the county Franklin and State of Ohio, have invented a new and useful Improvement in Cobble-Stone and Grout Pavements, of which the following is a full, clear, and exact description, reference being had to the annexed drawing, forming part of this specification.

10 The object of my invention is to provide a cheap pavement which will harden and solidify on exposure to moisture, and thus secure durability and that firmness of structure by which the noise commonly produced by vehicles passing over stone pavements shall be prevented.

The drawing represents a section of road-bed and pavement constructed according to my process.

My pavement is constructed in the following manner: When the road-bed A has been graded I spread gravel thereon to a depth of about four inches and roll the gravel with a heavy roller. I then spread about two inches of sand and pulverized slag upon the gravel, and upon this I lay the stones B with the small ends downward. The interstices between the stones are then filled to a depth of about two inches with a grout composed of the following ingredients: pulverized slag, thirty per cent.; clean river sand, thirty per cent.; rich lime, twenty per cent.; silica, six per cent.; Portland cement, six per cent.; ore-dust, eight per cent. Upon the grout I spread screenings to a depth of one or two inches more in order to hold the stones in position under the rammer and to make the pavement firm until the grout has time to harden. Before laying a course of grout the pavement or bed is always sprink-

led with water to furnish the required amount of moisture for making a mortar or cement. 40 When the screenings are spread and the work is properly rammed the pavement is again sprinkled with water, and the interstices between the stones are filled with another layer of grout to a level with the surface of the pavement. 45 A light coat of sand is then spread over the surface of the pavement, and on the following day the pavement will be ready for use.

With this construction the slag under the stone will become saturated with water, and will harden in course of time, like mortar, while the grout will form a more durable filling than the ordinary asphaltum pitch or coal-tar. The latter disintegrates and crumbles, and in a few years will become useless, while the grout improves with age and renders the pavement a solid stony mass. 55

I am aware that most of the above-named ingredients have been variously combined with pitch or asphaltum in forming paving compositions, and I therefore do not claim them, broadly. 60

Having thus described my invention, what I claim, and desire to secure by Letters Patent, is— 65

A pavement consisting of cobble-stones and a grout composed of pulverized slag, sand, lime, silica, Portland cement, and ore-dust, substantially as described, whereby the use of pitch or asphaltum may be dispensed with, as 70 set forth.

JOHN MURPHY.

Witnesses:

J. D. SULLIVAN,  
J. C. RICHARDS.